

June 29, 1965

H. MERKEL

3,192,139

METHOD FOR PRODUCING HYPERPURE GALLIUM

Filed April 19, 1961

2 Sheets-Sheet 1



Fig. 1

June 29, 1965

H. MERKEL

3,192,139

METHOD FOR PRODUCING HYPERPURE GALLIUM

Filed April 19, 1961

2 Sheets-Sheet 2



Fig. 2



Fig. 3

3,192,139

METHOD FOR PRODUCING HYPERPURE  
GALLIUM

Hans Merkel, Erlangen, Germany, assignor to Siemens-Schuckertwerke Aktiengesellschaft, Berlin-Siemensstadt and Erlangen, Germany, a corporation of Germany

Filed Apr. 19, 1961, Ser. No. 116,214

Claims priority, application Germany, Apr. 21, 1960,  
S 68,144

6 Claims. (Cl. 204—64)

My invention relates to a method and apparatus for producing hyperpure gallium.

Such gallium is needed mainly in the production of semiconducting gallium compounds such as GaP, GaAs, and GaSb, and also as a doping and contacting substance for semiconductor bodies. Hyperpure gallium is also used for example, in high-temperature thermometers, and in cooling systems where gallium serves as a liquid metal for heat-exchange purposes.

Various methods have become known for extreme purification of gallium. For example, it has been attempted to purify gallium metal by zone-pulling. The results are unsatisfactory. It is possible to purify gallium chloride  $\text{GaCl}_3$  by zone-pulling operations but the separation of gallium from the purified  $\text{GaCl}_3$  is difficult and not satisfactory for practical industrial application. This is mainly due to the fact that molten  $\text{GaCl}_3$  is electrically nonconductive. It is known to dissolve the purified compound in water, acid, or preferably in lyes, and to precipitate the metallic gallium electrolytically from the solution. This process, however, carries impurities from the solvent into the precipitated gallium. Further contamination is due to chemical attack upon the electrodes by the chlorine evolving at the anode. The electric current economy is relatively poor, and the electrolysis of aqueous gallium solutions takes place with violent liberation of gas at the electrodes.

It is therefore another, more specific object of my invention to provide a method for the production of hyperpure gallium which eliminates the above-mentioned difficulties and deficiencies.

According to the invention, I purify gallium by molten-bath electrolysis and use as an electrolyte a Ga(II)-halide previously subjected to extreme purification by zone-pulling in one or more passes.

The invention is based upon the observation that Ga(II)-halides are susceptible to extreme purification by zone-pulling. For example,  $\text{GaBr}_2$  can be purified in about 20 to 40 zone-pulling passes to such an extent that impurities are no longer discernible either spectroscopically or by the most sensitive known chemical methods of analysis. Molten Ga(II)-halides, in contrast to the trivalent gallium halides, are very good electric conductors. This is because Ga(II)-halides are ionic compounds of the type  $\text{Ga}^+(\text{GaX}_4)^-$  having a mono-valent gallium cation. The use of the Ga(II)-halides as the electrolyte for gallium purification by electrolysis of a molten or fused salt in accordance with my invention, is predicated upon the just-mentioned character of these compounds.

According to another feature of my invention, the above-described method is carried out in molten-salt electrolysis equipment whose electrodes consist of liquid gallium metal.

Examples of apparatus particularly well suitable for performing the method according to the invention are illustrated on the accompanying drawing by way of example.

FIG. 1 shows schematically an apparatus for single-stage processing;

FIG. 2 shows schematically another apparatus for two-stage processing; and

FIG. 3 is a single-stage apparatus according to the invention for large-quantity production of gallium.

The apparatus according to FIG. 1 comprises a vessel 1 for accomodating the electrolyte. The vessel 1 is mounted in a furnace schematically shown at 2 and consisting for example of an electric-resistance furnace. The electrode portions of the vessel are designed as U-shaped tubes, the anode tube is denoted by 3 and the cathode tube by 4. The current-supply conductors 5 and 6 are provided with small platinum tips 5a and 6a, for example of 0.3 mm. diameter, through which the current passes from the conductor to the liquid electrodes. The vessel portions 3, 1 and 4 are sealed by conical, ground closure caps 7, 8 and 9 respectively.

In performing the method of the invention, anode tube 3 is filled with impure gallium whereas the cathode tube 4 is filled with gallium of highest available purity, for example gallium already pre-purified by known purification methods.

It is preferable to use pre-purified gallium metal also in the anode tube rather than impure gallium as mentioned above. Particularly suitable for this purpose is gallium metal pre-purified in accordance with the method described in U.S. Patent 2,927,853. According to this method, the gallium metal, in form of droplets, is exposed, at a temperature between about 400 to about 1200° C., to a flow of nitrogen or ammonia gas.

The main vessel portion 1 is filled with the Ga(II)-halide electrolyte, for example  $\text{GaBr}_2$ , previously extremely purified by zone-pulling, the electrolyte forms an interface with the gallium electrodes. The electrolyte can be produced in known manner, for example by heating of commercially available gallium metal in a flow of nitrogen laden with bromine vapor. The resulting  $\text{GaBr}_3$  converts into  $\text{GaBr}_2$  by additional metallic gallium. The resulting  $\text{GaBr}_2$  can be rendered hyperpure, i.e. spectroscopically pure, by zone-pulling in about 20 to 40 zone passes.

The vessel portion 1 is heated to a temperature of approximately 190° C. by heating means 2. The electrolysis is preferably performed at a current density of 5 to 10 a./dm.<sup>2</sup> (amps per square decimeter). This results in the terminal voltage of 0.5 to 1 v. in apparatus according to FIG. 1. Metals, e.g. silver, copper, lead, etc., that are nobler than gallium and contained therein remain unchanged in the anode portion. Due to their high rate of diffusion, these nobler metals distribute themselves very rapidly throughout the entire quantity of the anode gallium, so that even after prolonged duration of the electrolysis, enrichment in these impurities does not occur in the vicinity of the anode surface. Although less noble metals, e.g. aluminum and zinc, enter anodically into solution along with gallium, only pure gallium is precipitated at the cathode. While the precipitation potentials of the particular metals is a factor, the high refining action is predominantly a consequence of the fact that the base metals enter into the anion complex of the electrolyte and therefore do not disturb the precipitation of pure gallium at the cathode. Thus, for example, anodically dissolved aluminum forms the negatively charged complex  $(\text{AlBr}_4)^-$ .

The quantitative analysis of the electrolysis shows that Faraday's law is strictly satisfied. That is, exactly 1 mole of gallium is converted by a quantity of electricity in the amount of 96,500 coulombs. This permits the conclusion that the electrolytic phenomena are determined by the electric charging, migration, and discharging of mono-valent Ga-cations. This is in harmony with the formulation of the Ga(II)-halides as being gallium(I)-

tetrahalogallates (III), i.e.  $\text{Ga}^+(\text{GaX}_4)^-$ , as ascertained in a different way and published recently. See Partington, "Textbook of Organic Chemistry," 6th edition (Macmillan and Co., London), page 816.

In conjunction with the production method of my invention, this result is of outstanding economical importance because the molten-salt electrolysis of the Ga(II)-halides yields the electrochemically possible maximum quantity of gallium, namely 2.6 g. Ga/ah. (grams of gallium per ampere hour). This quantity is exactly twice as large as would have to be expected on the basis of the simple formula  $\text{GaX}_2$  with bi-valent  $\text{Ga}^{++}$  cations.

Also economically important is the fact that with fused-bath (molten-salt) electrolysis, the refined gallium obtained utilizes 100% of the electric current. This is because the electric energy supplied to the system cannot be consumed by undesired secondary reactions, for example, gas development at the electrodes. This absence of gassing also permits performing the electrolysis in enclosed apparatus, thereby excluding the danger of contamination by atmospheric impurities.

The electrolysis equipment according to FIG. 1, suitable for producing relatively small gallium quantities up to about 50 g. Ga/24 hours, is preferably so dimensioned that the cathode space 4 is just filled with gallium at the termination of the 24-hour operating period. To withdraw the purified gallium, cap 9 is removed and the quantity of gallium metal equivalent to the gallium precipitated is withdrawn from the cathode space 4 by means of a pipette. The same quantity of impure gallium is added to the anode space 3.

#### Example 1

Commercially available gallium is used in the apparatus shown in FIG. 1.  $\text{GaBr}_2$  is used as the electrolyte. Both substances are pre-purified in accordance with the above-mentioned methods. The anode surface and the cathode surface amount to  $2.5 \text{ cm}^2$  each. The cell voltage is 0.5 volt. The electrolysis current is 0.25 amp. The vessel portion 1 was heated up to a temperature of  $190^\circ \text{ C}$ . After 24 hours 15.5 g. hyperpure gallium was obtained. The criterion of purity is described in the last paragraph of the specification.

According to another feature of the invention, the purification can be improved by performing the process in a plurality of steps, as already mentioned above. The embodiment of equipment shown in FIG. 2 is suitable for this purpose. The design of the individual stages essentially corresponds to the single-stage design according to FIG. 1. Shown between the two stages is an auxiliary electrode in a vessel portion 20. This auxiliary electrode makes it possible, in cooperation with the respective current sources provided for the two stages and in conjunction with an adjustable resistor, to control and regulate the current and voltage conditions of each individual cell independently of the other. However, the auxiliary electrode is dispensable for normal operation of the plant if so desired.

The apparatus according to FIG. 2 comprises an anode vessel 11, a cathode vessel 12, two vessel portion 13 and 14 for accommodating the electrolyte, and five ground covering caps 15, 16, 17, 18, 19 for vacuum-tightly closing and sealing the above-mentioned four vessel portions and the vessel portion 20 in which the auxiliary electrode is located. The current supply conductors 21, 22 and 23 are provided with small platinum tips for transferring the current to the respective gallium quantities. The current sources 24 and 25 for the two respective stages are connected in series with adjustable resistors 26 and 27 respectively. Each of the two circuits also comprises an ammeter 28 or 29, and a voltmeter 30 or 31.

The performance of the two-stage apparatus, in principle, is as described above with reference to the apparatus of FIG. 1. The purified gallium precipitated at the cathode side of the first stage constitutes the anode side of the

second stage in which the gallium is further purified and is precipitated at the cathode side of the second stage. In an analogous manner, the apparatus may be provided with any desired number of further stages.

#### Example 2

Commercial gallium and an electrolyte consisting of  $\text{GaBr}_2$  were used in the apparatus of FIG. 2. Both materials were prepurified as mentioned in Example 1. The anode surface per cell was  $7 \text{ cm}^2$ . The cathode surface per cell was  $1.75 \text{ cm}^2$ . At a voltage of 0.5 v. at the one cell and 0.9 v. at the other cell, an electrolysis current of 0.7 amp. adjusted itself. The two vessels with the electrolyte were kept at a temperature of  $190^\circ \text{ C}$ . The yield of 43.5 g. was obtained for 24 hours. Since in this example a two-stage purification was performed, the gallium produced was of even higher purity than the material of Example 1.

For producing large quantities of hyperpure gallium, it is necessary to provide electrolysis equipment that affords accommodating the largest feasible anode surface so that, for example, at anode-current densities between 5 and 10 a./dm.<sup>2</sup> correspondingly increased gallium throughputs are afforded at voltages between 0.5 to 1 v. In this case it is preferable to connect to the anode side of the electrolysis cell a gallium supply container with a level regulator, and to provide the cathode side with a collector vessel into which the purified gallium can drip continuously. For producing approximately 1 kg. refined gallium within 24 hours, an anode surface of approximately  $1.6 \text{ dm}^2$  is needed. The cathode surface is preferably smaller than the anode surface subdivided into several areas to obtain a favorable course of the current paths.

An example of such a design for large-scale production of gallium is illustrated in FIG. 3. The anode gallium and the electrolyte are located in an electrolytic cell 32. The cathode comprises two portions 33 and 34 which communicate with the cell 32 and with an end portion 36 of the cathode. The anode area is greater than the cathode area. The current supply can be effected for example by platinum tips that are fused into the vessel walls, such tips being indicated at 37 and 38. Located on the anode side of the apparatus is a gallium storage vessel 39 with a syphon tube 40 and a level regulator 41, the inlet opening is covered by a cap 42. The end portion 36 of the cathode is sealed by the ground cap 43 and provided with an overflow nipple 44. The cathodically precipitated gallium collects in a collector vessel 45 which is closed by sealing cap 46 which contains an air filter 47. The level regulator 41 permits adjusting the height of the anode gallium in the electrolytic cell and maintaining it constant. The cell 32 is located within an electric furnace whose heater winding is denoted by 48.

For the production of relatively small and medium throughputs of gallium, the electrolytic apparatus according to the invention are preferably made of glass or quartz-glass.

For larger throughputs, for example in equipment according to FIG. 3, recently developed quartz-glass-like materials which are particularly designed for larger dimensions can be used. This material is produced by a sintering or similar ceramic method and is commercially available under the trade name "Rotosil."

This material readily affords designing electrolytic cells, for example for 0.4 times  $2 \text{ m}^2 = 0.8 \text{ m}^2$  anode surface which furnish 50 kg. hyperpure gallium metal within 24 hours at 1 volt cell voltage and 800 a., thus requiring less than 20 kwh. expenditure in electrical energy.

$\text{GaCl}_2$ ,  $\text{GaI}_2$  can be used in lieu of  $\text{GaBr}_2$  in the same manner as that described above for  $\text{GaBr}_2$ . When using  $\text{GaCl}_2$ , the fact that an abrupt volume change takes place when the melting zone solidifies, must be taken into consideration when dimensioning the melting vessel.

The method according to the invention affords the production of gallium metal which is purer than 99.9999%. The known trace analysis methods (Dithizon method,

evaporation analysis, and others) furnish no indication of any foreign metals in this product. By thorough analytical investigation it has been found that any copper and lead impurities are reliably far below 10<sup>-5</sup>% and any zinc impurities reliably below 10<sup>-7</sup>%.

I claim:

1. The method of producing hyperpure gallium by electrolysis of a fused bath of electrolyte which comprises using gallium(II)-halides of the group consisting of chlorine, bromine and iodine as said electrolyte, said gallium(II)-halide being pre-purified by zone-pulling and using liquid gallium metal as electrodes.

2. The method of producing hyperpure gallium by electrolysis of a fused bath of electrolyte which comprises using gallium(II)-bromide,  $GaBr_2$ , as said electrolyte, said gallium(II)-bromide being pre-purified by zone-pulling and using liquid gallium metal as electrodes.

3. The method of producing hyperpure gallium by electrolysis of a fused bath of electrolyte which comprises using pre-purified gallium(II)-bromide as said electrolyte and liquid gallium metal as electrodes, said liquid gallium metal being pre-purified, at a temperature between about 400° C. and about 1200° C., by exposure, in the form of droplets, to a flow of nitrogen-containing gas.

4. The method of producing hyperpure gallium by electrolysis, which comprises zone-pulling gallium(II)-halides of the group consisting of chlorine, bromine and iodine to pre-purify said gallium(II)-halide, using said pre-purified gallium(II)-halide as a fused electrolyte for said electrolysis and liquid gallium metal as electrodes.

5. The method of producing hyperpure gallium by electrolysis of a fused bath of electrolyte which comprises using monovalent gallium cations extremely pre-purified by zone-pulling and liquid gallium metal electrodes.

6. The method of producing hyperpure gallium by electrolysis of a fused bath of electrolyte which comprises using monovalent gallium compounds of the group consisting of  $Ga[AlBr_4]$  and  $Ga[AlCl_4]$  as said electrolyte, said gallium compounds being pre-purified by zone-pulling and liquid gallium metal electrodes.

#### References Cited by the Examiner

##### UNITED STATES PATENTS

|    |           |      |           |         |
|----|-----------|------|-----------|---------|
| 15 | 1,842,254 | 1/32 | Driggs    | 204—64  |
|    | 2,500,284 | 3/50 | Heyrovsky | 204—219 |
|    | 2,927,853 | 3/60 | Merkel    | 75—84   |
|    | 2,991,235 | 7/61 | Ravier    | 204—64  |

##### FOREIGN PATENTS

|    |        |      |         |
|----|--------|------|---------|
| 20 | 72,710 | 1/30 | Sweden. |
|----|--------|------|---------|

##### OTHER REFERENCES

Jahresbericht Über Die Fortschritte der Chemie, Theil 1 (1888).

JOHN H. MACK, *Primary Examiner.*

JOHN R. SPECK, WINSTON A. DOUGLAS,

*Examiners.*